

# United States Patent Office

3,062,692

Patented Nov. 6, 1962

1

3,062,692

## AUSTENITIC STEEL GENERATOR RINGS AND STEEL THEREFOR

Samuel J. Manganello, Wilkins Township, Allegheny County, and Matti H. Pakkala, Pleasant Hills Borough, Pa., assignors to United States Steel Corporation, a corporation of New Jersey

No Drawing. Filed Nov. 4, 1959, Ser. No. 850,792  
6 Claims. (Cl. 148—38)

This invention relates to generator rings and steels therefor capable of developing high yield strengths by cold working and aging coupled with sufficient ductility to permit large amounts of cold work and more particularly to generator rings and forgings having such properties along with a grain size no larger than ASTM #4.

So-called "generator rings" or "retaining rings" used as coil supports in generator rotors must be formed of austenitic, i.e. nonmagnetic, steels to avoid electrical losses. It is necessary that these rings possess high yield point in excess of 125,000 p.s.i. (0.2% offset) which require that the rings after forging and heat treating must be warm or cold expanded 25% or more to develop the required strength limit. These rings are subjected to rigid inspections because of the serious nature of failure in use. Ultrasonic inspection is one of the preferred types of inspection but this cannot be used satisfactorily on steels having a grain size larger than ASTM #1.

It is accordingly an object of the present invention to provide austenitic generator ring steels having a grain size no larger than ASTM #4 along with good hot and cold forging properties.

The foregoing and further objects will be apparent from the following specification.

We have discovered that the desired combination of properties can be achieved with a steel composition containing:

.60 to .80% carbon  
8.00 to 10.00% manganese  
.20 to .60% silicon  
6.00 to 7.00% nickel  
4.00 to 5.00% chromium  
.30 to .60% columbium

with the balance substantially iron and other elements in amounts which are not harmful to the properties.

As a specific example, steel of the following composition was treated in accordance with our invention:

0.70% carbon  
9.00% manganese  
.035% phosphorus  
.015% sulphur  
0.50% silicon  
6.50% nickel  
4.25% chromium  
0.010% aluminum  
0.010% nitrogen  
0.30% columbium

with balance substantially iron.

Ring specimens of this steel were heated to 2000° F. for 2 hours and air cooled. After heating and cooling, the specimens had a grain size of 5-6 according to the ASTM chart. One specimen was cold expanded 25% and the other 30%. The 30% expanded steel was then

2

subjected to an aging treatment at 600° F. for 2 hours. The results were as follows:

|    | 5  | Cold Worked, percent     | Yield Strength (0.02% offset), p.s.i. | Yield Strength (0.2% offset), p.s.i. | Tensile Strength, p.s.i. | Elongation in 2", percent | Reduction of Area, percent |
|----|----|--------------------------|---------------------------------------|--------------------------------------|--------------------------|---------------------------|----------------------------|
| 25 |    |                          | 83,900                                | 143,250                              | 168,500                  | 39.5                      | 41.6                       |
| 30 |    |                          | 102,150                               | 154,850                              | 173,900                  | 31.0                      | 38.1                       |
| 10 | 10 | Cold Worked 30% and Aged | 147,800                               | 156,400                              | 170,400                  | 32.0                      | 40.6                       |

These tests indicate that the steel of our invention may be cold expanded 25 to 30% to obtain the desired tensile strength and 0.2% offset yield strength. Considerable improvement in the .02% offset yield is obtained by aging along with minor improvements in .2% offset yield, tensile strength, elongation and reduction of area. The aging should be in the range of 500 to 650° F. for sufficient time to achieve uniformity of temperature.

The grain size above stated is a true inherent grain size and remains substantially the same after different solution temperatures as can be seen from the following tabulation.

|  | 25 | Solution temperature: | ASTM grain size |
|--|----|-----------------------|-----------------|
|  |    | 1800° F.              | 6-7             |
|  |    | 2000° F.              | 5-6             |
|  |    | 2200° F.              | 4-5             |

30 While we have shown and described one specific embodiment of our invention, it will be understood that this embodiment is merely for the purpose of illustration and description and that various other forms may be devised within the scope of our invention, as defined in the appended claims.

We claim:

40 1. A cold expanded austenitic steel generator rotor coil support retaining ring characterized by a grain size no coarser than ASTM #4 containing .60 to .80% carbon, 8.00 to 10.00% manganese, .20 to .60% silicon, 6.00 to 7.00% nickel, 4.00 to 5.00% chromium and .30 to .60% columbium with the balance iron and other elements in amounts which do not have a harmful effect on the properties.

45 2. An austenitic steel generator rotor coil support retaining ring characterized by a grain size no coarser than ASTM #4 and by having been cold expanded over 25% containing .60 to .80% carbon, 8.00 to 10.00% manganese, .20 to .60% silicon, 6.00 to 7.00% nickel, 4.00 to 5.00% chromium and .30 to .60% columbium, balance substantially iron.

50 3. A method of producing austenitic steel generator rotor coil support retaining rings characterized by a grain size no coarser than ASTM #4 and 0.2% yield strength greater than 125,000 p.s.i. comprising forming a ring of steel containing .60 to .80% carbon, 8.00 to 10.00% manganese, .20 to .60% silicon, 6.00 to 7.00% nickel, 4.00 to 5.00% chromium and .30 to .60% columbium, balance substantially iron, and cold expanding 60 said ring at least 25%.

4. A method of producing austenitic steel generator rotor coil support retaining rings characterized by a grain size no coarser than ASTM #4 and 0.2% yield strength greater than 125,000 p.s.i. comprising forming a ring of steel containing .60 to .80% carbon, 8.00 to 10.00% manganese, .20 to .60% silicon, 6.00 to 7.00%

nickel, 4.00 to 5.00% chromium and .30 to .60% columbium, balance substantially iron, cold expanding said ring between 25% and 30% and then aging it at a temperature between 500 and 650° F.

5. An austenitic steel characterized by good cold formability and a grain size no coarser than ASTM #4 containing .60 to .80% carbon, 8.00 to 10.00% manganese, .20 to .60% silicon, 6.00 to 7.00% nickel, 4.00 to 5.00% chromium and .30 to .60% columbium, balance substantially iron.

10. 6. An austenitic steel characterized by being hardenable by cold working and aging and having a grain size no coarser than ASTM #4 in the hardened condition,

said steel containing about .70% carbon, 9.00% manganese, .50% silicon, 6.50% nickel, 4.25% chromium, .010% aluminum, .010% nitrogen and .30% columbium, with the balance substantially iron.

References Cited in the file of this patent

UNITED STATES PATENTS

|           |           |       |               |
|-----------|-----------|-------|---------------|
| 1,561,306 | Brace     | ----- | Nov. 10, 1925 |
| 1,574,782 | Becker    | ----- | Mar. 2, 1926  |
| 2,449,023 | Thornton  | ----- | Sept. 7, 1948 |
| 2,859,149 | Straumann | ----- | Nov. 4, 1958  |

UNITED STATES PATENT OFFICE  
CERTIFICATE OF CORRECTION

Patent No. 3,062,692

November 6, 1962

Samuel J. Manganello et al.

It is hereby certified that error appears in the above numbered patent requiring correction and that the said Letters Patent should read as corrected below.

Column 1, line 28, for "ASTM #1" read -- ASTM #4 --;  
column 2, line 29, for "22000° F." read -- 2200° F. --.

Signed and sealed this 9th day of April 1963.

(SEAL)

Attest:

ESTON G. JOHNSON

Attesting Officer

DAVID L. LADD

Commissioner of Paten